

## UNITED STATES PATENT OFFICE

1,976,027

## TRANSPARENT SHEET MATERIAL

Edouard M. Kratz, Chicago, Ill., assignor to  
 Marsene Products Co., Gary, Ind., a corpora-  
 tion of Illinois

No Drawing. Application July 8, 1927,  
 Serial No. 204,422

8 Claims. (Cl. 91—68)

This invention relates to transparent sheet material and more particularly to a coated gelatine composition sheet adapted for wrapping purposes.

5 Heretofore, gelatine has been considered unsuitable for the manufacture of waterproof wrapping material, because, although the gelatine may be rendered insoluble by the use of tanning agents, a tanned gelatine sheet will still permit 10 the passage of moisture through it. Cellophane (cellulose xanthate) is also objectionable in this respect, since it takes water only about 10 seconds to pass through a sheet of cellophane .001 inch thick. Sheets of cellulose nitrate or acetate 15 are in general waterproof but rather expensive of manufacture.

It is therefore an object of this invention to provide an inexpensive transparent, flexible wrapping material made of gelatine or gelatine 20 composition as a base and having a waterproof coating of a cellulose ester or mixture of esters.

Other and further important objects of this 25 invention will become apparent from the disclosures in the following description and appended claims.

The present invention consists in coating a straight gelatine film or a film made from gelatine and sulphonated castor oil, as disclosed in my co-pending application, Serial No. 10,962, 30 filed February 21, 1925, with a cellulose ester, such as cellulose nitrate or acetate, or a mixture of the two. The gelatine or gelatine-sulphonated oil composition may be formed as a film upon any suitable surface from which it may be readily stripped when dry. I prefer to use the coated 35 fabric surface or belt disclosed in my co-pending application, Serial No. 11,335, filed February 24, 1925, wherein the surface is formed of baked drying oils. If a gelatine composition base is to be used, I prefer a composition such as disclosed 40 in my co-pending application, Serial No. 10,962, comprising approximately 60 to 85% glue and 15 to 40% sulphonated castor oil. Preferably no tanning agent is used.

45 The gelatine, or gelatine composition film is then coated with cellulose nitrate, or acetate, or a mixture of the two, either on one or both sides of the film. Cellulose acetate being non-inflammable, it is possible to prepare a mixture 50 of the two esters wherein the cellulose acetate contact is sufficiently high to render the mixture also non-inflammable.

The coating is preferably effected by means of a doctor. A surplus of the coating material dissolved in a volatile solvent is deposited on the

traveling film ahead of the doctor and the excess scraped off by the doctor, thus leaving a uniform thin coating on the film. The evaporation of the solvent is preferably effected while the film is passing under tension over a curved surface, so as to prevent the edges of the film from curling. Obviously, the process may be made continuous if desired.

Where the sheet material is to be used for making bags or for some wrapping purposes, it is preferable to coat the gelatine base film on but one side. The sheet material is then self sealing, since the application of moisture to the uncoated surfaces render them adhesive. For other purposes the sheet may be coated on both sides.

While I do not wish to limit the composition of the sheet material to any specific proportions, the following will serve to illustrate my preferred composition:

|                                        | Per cent | 75 |
|----------------------------------------|----------|----|
| Ethyl acetate                          | 14       |    |
| Butyl acetate                          | 27       |    |
| Toluene                                | 14       |    |
| Cellulose nitrate and acetate (1 to 2) | 23       |    |
| Alcohol (denatured #1)                 | 6        | 80 |
| Benzene                                | 3        |    |
| Dammar gum                             | 8        |    |
| Tri-cresyl-phosphate                   | 5        |    |
|                                        | 100      | 85 |

In place of tri-cresyl-phosphate, any suitable plasticizer may be used. Other satisfactory solvents for the cellulose esters will also occur to those familiar with the art.

I am aware that numerous details of the process may be varied through a wide range without departing from the principles of this invention and I, therefore, do not purpose limiting the patent granted hereon, otherwise than necessitated by the prior art.

I claim as my invention:

1. A transparent self-sustaining sheet comprising a gelatinous base having a water proof coating of cellulose nitrate, cellulose acetate and tri-cresyl phosphate.

2. A transparent self-sustaining sheet comprising a gelatinous base having a water proof coating of cellulose nitrate, cellulose acetate, tri-cresyl phosphate and dammar gum.

3. A transparent self-sustaining sheet comprising a base formed of gelatine and sulphonated castor oil and having a water proof coating comprising one part cellulose nitrate to two parts celu-

lose acetate with small amounts of tri-cresyl phosphate and dammar gum.

4. An integral, transparent wrapping sheet comprising a thin film of gelatine as a base, a coating of cellulose nitrate applied to each face of said film and having incorporated therein a plasticizer, the cellulose nitrate coating being integrally united with the gelatine on each side thereof and the thickness of said film and coating respectively being such that said resultant wrapping sheet will be flexible, transparent and waterproof and adapted to conform readily to the shape of packages and the like without cracking or separating.

15 5. An integral, transparent wrapping sheet comprising a thin film of gelatine as a base, a coating of cellulose nitrate applied to each face of said film and having incorporated therein tri-cresyl phosphate.

20 6. An integral transparent wrapping sheet of the character described consisting of a thin film of a protein substance as a base, a coating of cellulose nitrate applied to each face of said film and having incorporated therein a non-hygroscopic bonding agent (other than castor oil) in such a quantity as to cause the cellulose nitrate coating to become integrally united with the protein film on each side thereof, the thickness of the said film and coating respectively being such as that said resultant wrapping sheet will be tough, pliable, transparent, moisture, grease and water proof and adapted to readily conform to the shape of packages and the like without cracking or separating.

25 30

the shape of packages and the like, without cracking or separating.

7. An integral transparent wrapping sheet of the character described consisting of a thin film of a protein substance as a base, a coating of cellulose nitrate applied to each face of said film and having incorporated therein a non-hygroscopic bonding agent (other than castor oil) in such a quantity up to 80% by weight of the dried coating of cellulose nitrate as to cause the cellulose nitrate coating to become integrally united with the protein film on each side thereof, the thickness of the said film and coating respectively being such as that said resultant wrapping sheet will be tough, pliable, transparent, moisture, grease and water proof and adapted to readily conform to the shape of packages and the like without cracking or separating.

8. An integral transparent wrapping sheet comprising a thin film of protein material as a base, a coating of a cellulose derivative selected from the group consisting of cellulose nitrate and a mixture of cellulose nitrate and cellulose acetate applied to said film and having incorporated therein a plasticizer, the cellulose derivative coating being integrally united with the base, the thickness of said base and coating being such that the said resulting wrapping sheet will be flexible, transparent, and waterproof and adapted to conform readily to the shape of packages and the like without cracking or separating.

EDOUARD M. KRATZ.

35

40

45

50

55

60

65

70

75